

## UNITED STATES PATENT OFFICE.

NOAK VICTOR HYBINETTE, WILMINGTON, DELAWARE.

## PROCESS OF PRODUCING NICKEL ALLOYS.

No Drawing.

Application filed September 23, 1922. Serial No. 589,997.

This invention relates to an improved method of producing nickel alloys from which sound castings can be obtained.

Nickel has a decided affinity for gases and 5 absorbs them readily when in a molten state. As a result, the castings produced from the molten nickel are unsound or spongy due to the setting free of the absorbed gas on cooling. This affinity for 10 gases is also noticed in nickel alloys, particularly when the nickel is fairly high in amount. It is known that carbon and silicon tend to reduce such an affinity, but for 15 many purposes both nickel and nickel alloys are more valuable without the addition of these elements.

I have discovered that highly oxidized (i. e. containing appreciable quantities of oxide) nickel and nickel alloys, such as 20 nickel-iron alloys are unable to hold gases in solution, at least not to such an extent as to be practically noticeable. I have further discovered that if the oxidized molten nickel or alloy is covered and protected with 25 a slag and treated with a deoxidizer other than carbon, the molten nickel or alloy can be deoxidized without the formation of gas so that a sound casting can be produced free from carbon. This method of procedure is 30 particularly advantageous in making malleable nickel alloys and ferro-nickel alloys such as chromium-nickel-iron alloys for rolling or for casting.

In producing such alloys, the pure nickel, 35 or the mixture containing nickel or nickel and iron, is melted in a reverberatory furnace under oxidizing conditions so as to produce a metal containing about .02% of oxygen. This oxidizing treatment renders 40 the molten metal free or practically free from gases so that a sample of the metal, cast in an open mold, shows no gas and gives a casting which is smooth on the surface and without signs of sponginess in the grain. 45 If a sample cast in this way rises and the grain is full of gas bubbles then the oxidizing has been insufficient. When the proper degree of oxidizing has been reached, the molten metal should be covered with a fairly 50 neutral slag of silicates such as the silicates of lime, magnesia and alumina, but with no large proportion of iron, nickel, etc. in the slag. The slag may be present during the oxidizing operation or it may be added 55 near the end of the operation. The oxidizing operation not only frees the molten

metal from gases but it also removes to a greater or less extent such impurities as carbon, silicon, etc.

When a test of the molten metal shows 60 that it has been oxidized sufficiently and is free from gas, a deoxidizer is then introduced under the slag. The deoxidizer should be one which does not itself form gaseous products but which forms non-gaseous 65 oxides. I prefer to use metallic aluminum for this purpose, but other deoxidizers free or nearly free from carbon may be used, for example, manganese, silicon, magnesium or mixtures of these with aluminum, etc. 70 With aluminum the deoxidizing is carried to as nearly as possible the neutral point so that no oxygen remains and no aluminum is present. This point can easily be reached. When the molten metal has been deoxidized 75 in this way, I then add the other ingredients of the alloy such as ferro-chromium, etc. If these added ingredients contain carbon, no objectionable carbon monoxide is formed because of the freedom of the bath from 80 oxygen and the resulting alloys can accordingly be cast to give sound castings.

In order to make malleable nickel or malleable alloys of nickel, there is introduced into the alloy, before casting, a small amount 85 of magnesium, either as pure magnesium in the case of alloys containing less than 40% of iron, or as an alloy of magnesium in alloys containing more iron. If the highest degree of malleability is unnecessary, magnesium may be dispensed with in alloys containing less than 60% of nickel, provided manganese, chromium, etc. are present.

The present invention is particularly advantageous in producing a superior quality 95 of malleable nickel free from carbon inasmuch as any carbon present originally in the nickel is removed by the oxidizing treatment, and the subsequent deoxidizing does not introduce carbon into the metal. The 100 invention is also particularly advantageous in producing ferro-alloys such as chromium-nickel-iron alloys low in carbon, since the ferro-nickel to which the alloying metals are added is itself free from carbon and only 105 such carbon is present in the final alloy as is added with the alloying metals.

Alloys of chromium, nickel and iron can thus be made by forming a ferro-nickel bath in the manner above described and then 110 adding ferro-chromium to the bath. Since the ferro-nickel bath is itself free from car-

bon, the only carbon present is that added with the ferro-chromium, and, where the amount of ferro-chromium added is not too great, a high carbon ferro-chromium can be used, without introducing an objectionable amount of carbon into the alloy. For example, in making alloys containing from 10 to 15% of chromium, around 30 to 35% of nickel and the remainder for the most part iron, the chromium can be supplied in the form of the cheap ferro-chromium containing around 5 to 6% of carbon and the resulting alloy will contain less than 1% of carbon. Where it is important to have a lower carbon content, this can be regulated by regulating the amount of carbon added with the ferrochromium. The freedom from carbon of the ferro-nickel bath to which the ferrochromium is added makes it possible to use a less expensive grade of ferrochromium with a higher carbon content than would be possible if the ferro-nickel were not itself free from carbon. The alloys thus produced can be used as heat resisting alloys, or for heat resisting castings, or for other purposes.

In referring to a nickel-containing bath in the appended claims or to a molten bath of the nickel or nickel alloys, I mean a bath such as is hereinbefore described of metallic nickel, a nickel-iron alloy bath, etc., which are to be used for making castings or which are to be treated with an alloying metal for the manufacture of nickel-containing alloys suitable for casting.

I claim:

1. The method of producing nickel alloys which comprises subjecting a nickel-containing bath to an oxidizing treatment, deoxi-

dizing the oxidized bath with a deoxidizer forming a non-gaseous oxide, and adding an alloying metal or metals to the deoxidized bath.

2. The process of treating nickel or nickel alloys which comprises subjecting a molten bath of the same to an oxidizing treatment, and deoxidizing the oxidized bath with a deoxidizer forming a non-gaseous oxide.

3. The method of producing casting of nickel and nickel alloys which comprises subjecting a molten bath of the same to an oxidizing treatment, deoxidizing the oxidized bath with a deoxidizer forming a non-volatile oxide, and casting the resulting metal.

4. The method of treating nickel and nickel alloys which comprises subjecting a molten bath of the same to an oxidizing treatment to remove gases and readily oxidizable impurities therefrom, protecting the oxidized bath by a slag nearly neutral in character and adding a deoxidizer which forms a non-gaseous oxide to the bath while protected by the slag.

5. The process according to the preceding claim in which an alloy metal or metals is or are added to the deoxidized molten bath.

6. The method of producing chromium-nickel-iron alloys which comprises subjecting a molten bath of nickel or nickel and iron to an oxidizing treatment, a deoxidizing the oxidized bath with a deoxidizer forming a non gaseous oxide, and adding ferrochromium to the deoxidized bath.

In testimony whereof I affix my signature.

NOAK VICTOR HYBINETTE.